

A. Hamar.

Street,  
3 Streets.

## Converting Cast Iron into Steel.

№ 86,536.

Patented Feb. 2, 1869.



*Witnesses,*

Warrupper  
J. A. Baylow  
Baltt De Long.

Inventor  
Alexander Hamer  
11-8-1944

Alexander Stanner  
by his attorney  
W. D. Baldwin

A. Hamar.

Sheet 2,  
3 Sheets.

Converting Cast Iron into Steel.

Inv. 80,536.

Patented Feb. 2, 1869.

Fig. 2



Witnesses  
J. D. Payton  
Batty De Long

Inventor  
Alexander Hamar  
by his Atty  
W. D. Baldwin

A. Hamar.

Sheet 3,  
3 sheets.

Converting Cast Iron into Steel.

No 86,530.

Patented Feb. 2, 1869.



Witnesses  
J. L. Peyton  
Baltus De Long.

Inventor  
Alexander Hamar  
by his son  
W. D. Baldwin

# United States Patent Office.

ALEXANDER HAMAR, OF PHILADELPHIA, PENNSYLVANIA.

Letters Patent No. 86,536, dated February 2, 1869.

## IMPROVED METHOD OF CONVERTING CAST-IRON INTO STEEL.

The Schedule referred to in these Letters Patent and making part of the same.

To all whom it may concern:

Be it known that I, ALEXANDER HAMAR, of the city and county of Philadelphia, in the State of Pennsylvania, have invented a new and improved Method of Converting Cast-Iron into Steel, of which the following is a full, clear, and exact description.

The object of my invention is to convert cast-iron into steel by a continuous operation.

The first part of my invention relates to the furnace in which the cast-iron to be converted into steel is melted; and my improvement consists in forming a bed, or hearth, for the furnace, of a mixture of nitrate of soda, one volume; pulverized charcoal, five volumes; slaked lime, five volumes. These ingredients are to be covered with a layer, half an inch in depth, of pulverized ilmenite, magnetite, or Franklinite, mixed with one-fourth its volume of slaked lime, made into paste with water.

The next part of my invention consists in combining a furnace to melt the iron, an insulated ladle to receive the melted metal from the furnace, a stack, through which the metal flows, an electric current acting on the flowing metal, and a converting-furnace.

My invention further consists in forming a bed in the ladle, of the following ingredients: alkaline nitrates, two parts; peroxide of manganese, one part; carburets, three parts.

The next part of my invention consists in combining a reverberatory furnace with a stack, through which the melted metal falls, and within which it is exposed to a blast, so that the stack shall serve as a chimney for the furnace.

My invention further consists in combining two or more fires with a reverberatory furnace, and with a showering-stack, which also serves as a common chimney for the fires, as hereinafter set forth.

In the accompanying drawings, which show convenient apparatus for carrying out my invention—

Figure 1 is a view, partly in section and partly in elevation, of a single converting-furnace and separate chimney;

Figure 2 is a vertical section through the converting-furnace and stack; and

Figure 3, a view of my improved apparatus, adapted to a double converting-furnace, and a stack, without a chimney.

The bottom of the furnace A is covered with a bed of nitrate of soda, one volume; pulverized charcoal, five volumes; slaked lime, five volumes. This mixture is covered with a layer, about half an inch deep, of pulverized ilmenite, magnetite, or Franklinite, mixed with one-fourth its volume of slaked lime, made into paste with water.

When dry, the furnace is charged with pig-iron and coal, in the usual way.

At suitable periods, the molten metal is run through a trough, a, into a ladle, B, electrically insulated, in any

proper well-known way, and connected with the negative pole of a strong electric battery, by a wire, a.

I form a bed in this ladle, of two parts of alkaline nitrates, one part of peroxide of manganese, and three parts of carburets. As the action of these ingredients often causes ebullition of the iron, I hinge a cover, B, on the ladle, so that it may be tipped to one side, as shown in fig. 3. This cover is of the shape of an inverted funnel, and is open at the top, to allow the gases to escape from the ladle.

A spout, b, conducts the melted iron into a stack, C, into which it falls, being scattered into spray by a cone, D, secured on suitable bars, e, some distance below the top of the stack, and suitably protected from heat by fire-clay, or equivalent means.

This cone may be so constructed as to be raised or lowered, to regulate the scattering of the metal, (and also the length of time the metal is exposed to the current,) and is perforated, so as to receive the other or positive pole of the battery, the wire p of which must of course be suitably insulated.

It will be seen that, by my mode of construction, the current of falling metal itself forms a connecting-link between the two poles of the battery.

The stack, C, in this instance, is formed of an outer casing, E, of iron, with an internal lining, e', of fire-brick, or brick so arranged as to leave an annular space, e'', between them.

This space serves as a blowing-chamber, through which a high-pressure blast of compressed air is forced into the stack, by numerous openings, f, at different elevations.

The hydrogen of the furnace, or the oxygen of the blast, encounters the falling current of metal just as it is chemically separated from its impurities by the electric current, and immediately unites with the carbon, forming carburetted hydrogen or oxygen, (as the case may be,) which, by its combustion, destroys or eliminates the other impurities of the iron.

In figs. 1 and 2, a fire-place, G, is shown, as arranged near the stack.

The fuel is placed on a grate, h.

Mingled jets of steam and air are introduced into the fire-place, below the grate, through pipes I i, from any proper apparatus.

The oxygen of the steam is consumed by the fire, and the remaining products of combustion (mainly carburetted hydrogen) pass over into the reverberatory furnace O, being mingled, at the bridge j, with jets of air, entering through apertures, K K, in the fire-chamber, by which means an intense heat is produced.

The draft can be regulated to any desired velocity, by valves on the inlet pipes I i, L l, and by the damper M on the chimney.

The hearth O is covered with a layer composed of a mixture of charcoal-dust, oxide of manganese, and a small quantity of slaked lime. Pig-iron is laid on this

bed, and melted by the heat produced, as above described.

The products of combustion escape up the stack C, through the trough K, by which the purified iron descends into the furnace O, and keeps the stack heated.

The iron, as it flows from the stack, is decarbonized, and minglest with the melted iron on the hearth O, and the mixture of these two produces steel of good quality, which is cast into ingots in the usual way.

If the metal on the hearth is too highly carbonized, it is decarbonized by being exposed to the blast a sufficient length of time. If not carbonized enough, a few pieces of carbonized iron are thrown in and melted.

In fig. 3, I have shown a modification of the apparatus shown in figs. 1 and 2. The modification consists in arranging two or more fires, G, around a central reverberatory furnace, O, placing the stack C over the furnace, and using this stack alone as the chimney. By this means, I am enabled to reduce the cost of the works, to economize fuel, and to increase the working-capacity of the furnace materially.

What I claim as my invention, and desire to secure by Letters Patent, is—

1. The combination of nitrate of soda, charcoal, slaked lime, and ilmenite, magnetite, or Franklinite, substantially as set forth, to form the bed of the melting-furnace.

2. The combination of a melting-furnace, an insulated ladle, a showering-stack, an electric current, and a converting-furnace, substantially as set forth.

3. The bed for the ladle, composed of alkaline nitrates, peroxide of manganese, and carburets, substantially as set forth.

4. The combination of a reverberatory or converting-furnace with a showering-stack, substantially as set forth.

5. The combination, substantially as set forth, with two or more fires, of a reverberatory or converting-furnace and a showering-stack, through which the molten metal and the products of combustion pass.

In testimony whereof, I have hereunto subscribed my name.

A. HAMAR.

Witnesses:

WM. B. DAYTON,  
TH. PRATT POTTS.